

## UNITED STATES PATENT OFFICE

SUMNER REDWAY MASON, OF WILMETTE, ILLINOIS, ASSIGNOR TO WESTERN ELECTRIC COMPANY, INCORPORATED, OF NEW YORK, N. Y., A CORPORATION OF NEW YORK

## METHOD OF TREATING METALLIC SURFACES

No Drawing.

Application filed September 12, 1928. Serial No. 305,618.

This invention relates to a method of treating metallic surfaces, and more particularly to a method of coating sherardized surfaces to improve their appearance.

5 On account of the dark color of sherardized surfaces, they are not suitable for exposed parts where appearance is of importance, which fact has in the past limited the application of sherardizing to such parts as

10 were not exposed to view.

An object of the present invention is a simple and inexpensive process to impart to sherardized surfaces a pleasing appearance.

The object of the invention is accomplished

15 by the provision of a cyanide and caustic soda solution containing cadmium in which the sherardized parts to be treated are immersed, which results in the formation of a thin coating of cadmium on the sherardized

20 surfaces.

The invention will be more fully understood from the following description.

In the practice of the invention a bath is formed, the preferred constituents and proportions of which are as follows:

|                   |           |
|-------------------|-----------|
| Water             | 250 c. c. |
| NaCN              | 60 g.     |
| NaOH              | 30 g.     |
| CdCO <sub>3</sub> | 10 g.     |

The proportions of the above ingredients may be considerably varied, depending upon the nature of the work to be finished, the thickness of cadmium coating desired, and various other factors, as will be apparent to those skilled in this art. It will also be obvious to those skilled in the art that certain substitutions may be made in the ingredients listed above. Thus, instead of cadmium carbonate, the chloride or other salt may be used; instead of the sodium cyanide; potassium or other cyanide may be used; or cadmium cyanide may be used to take the place of all of the cadmium carbonate and a part of the sodium cyanide.

The bath being preferably at a temperature of about 80° C., the sherardized parts are introduced therein by any suitable dipping means, and kept in the solution for one minute or such time as is found by experience to be sufficient to produce the desired coating. No external electromotive force need be applied, since the zinc, being above cadmium in the electromotive series, will displace the cadmium from the solution, forming an even electrolytic deposit of cadmium.

This treatment forms a pleasing white coating on the parts which greatly improves their appearance, and at the same time increases the rust-proofing effect of the zinc. Because of the fact that no electromotive force need be applied, the process may be carried out very economically.

## What is claimed is:

A method of brightening a sherardized surface, which consists in immersing the surface for about one minute in a bath containing the following ingredients in substantially the following proportions; water, 250 cubic centimeters; sodium cyanide, 60 grams; sodium hydroxide, 30 grams; and cadmium carbonate, 10 grams; the temperature of the bath being substantially 80° C., thereby causing the deposition of a thin layer of cadmium upon the surface without the imposition of an external electromotive force.

In witness whereof, I hereunto subscribe my name this 27th day of August, A. D. 1928.

SUMNER REDWAY MASON.

80

85

90